

1

3,079,213

ANTIMICROBIAL TREATMENT OF ORGANIC MATERIALS AND COMPOSITION THEREFOR  
Meyer Mendelsohn, New York, and Carl Horowitz, Brooklyn, N.Y., assignors, by mesne assignments, to Yardney International Corp., New York, N.Y., a corporation of New York  
No Drawing. Filed Dec. 11, 1959, Ser. No. 858,871  
11 Claims. (Cl. 8—115.5)

The present invention relates to a treatment of textiles and textile fibers of natural or synthetic origin, cellulosic or plastic resinous sheets, and similar organic materials in a manner imparting to them antimicrobial properties. This application is a continuation-in-part of our applications Ser. No. 548,253, filed November 21, 1955, Ser. No. 738,697, filed June 2, 1958, and Ser. No. 760,857, filed September 15, 1958, all now abandoned.

It is known that zinc and certain of its compounds are highly active against a wide spectrum of micro-organism. Heretofore, however, it has been difficult to utilize this property in industrial processes such as the manufacture of paper, textiles and the like where the presence of substantial quantities of free zinc or zinc oxide would be objectionable and where, up to now, no practical way had existed for maintaining a small percentage of zinc firmly attached to the material so as to retain its effectiveness during normal use, washings and so forth.

An object of the invention is to provide a process for virtually permanently fixing a small quantity of zinc in the molecular structure of cellulosic, proteinaceous and other organic materials such as, for example, wood, paper, cotton, linen, rayon, wool, silk natural bristles, hides, cellulosic sheets and films, sponges casein fibers and films, gelatin in foam or film form, and various thermoplastic resin such as polyamide (e.g. nylon) and polyester fibers and sheets.

Another object of the invention is to provide a novel chemical composition for use in such process.

It is also an object of the invention to provide a treatment for the purpose described which can be carried out at only moderately elevated bath temperatures, thus enabling the processing of heat-sensitive fabrics and the like.

A further object is to provide, as a novel industrial product, an article of commerce made of one or more of the aforescribed organic materials and treated in such manner as to be resistant to micro-organisms without being toxic or irritating to humans.

It is known to treat cotton fibers with a solution of urea and a zincate of sodium or potassium for the purpose of reducing shrinkage. In this known process, operating under conditions of very high alkalinity, the zinc compound remains in contact with the fabric for only a short period and is then washed out. The process of the present invention takes place in a considerably less alkaline or slightly acidic medium and, while employing urea or some other source of amine groups as a fixing agent, utilizes the presence of a sequestrant or chelating agent to form a zinc complex which is readily taken up by the molecule of the organic material to be treated.

The process according to the invention, accordingly, involves the steps of mixing together a water-soluble zinc salt, a chelating agent and an aminating agent and forming from this mixture an aqueous solution in which the organic material to be treated may be immersed until the molecules have taken up the zinc sequestrant complex. It should be noted that the aminating or fixing agent may be added to the original solution or may be applied to the treated material as a second step. Advantageously, a wetting agent or detergent and a buffering agent are also included in the solution so constituted.

2

The organic materials so treated are rendered resistant to bacteria so as not only to be safe from destruction by such organisms but also to be no longer a carrier of disease-bearing microbes. Frequently, the treated materials also appear resistant to mildew-causing organisms and have improved physical strength. Finished garments or similar industrial articles may be treated as well as fibers and fabrics.

While it has been known in the past to coat various materials with antimicrobic substances, such coatings have had several severe drawbacks including toxicity, allergenicity, and dye-destructiveness. Various forms of iodine, mercury, and organo-halides have proved to be either fugitive, toxic or prone upon repeated use to cause a high incidence of allergic reaction. Moreover, each of the above has affected either the dye structure or the substantiveness of the base material to dyes. Fabrics treated with such types of materials have been noted to dye with difficulty, and often not at all, to fade with time, or to change hue when exposed to actinic rays. In contrast, the compounds of this invention are formed within the polymeric chain and are, therefore, an integral part of the structure of the polymeric material. Moreover, since the treatment adds reactive groups to the molecule, it has been noted that the polymeric organic materials thus modified dye with ease and the colors are at least as intense as those achieved in the untreated fabrics.

An important advantage of the process of the invention is that since the active complex is in chemical combination with and directly incorporated into the polymeric structure, it resists removal from the polymeric material. It has been found that fabrics so treated retain their antimicrobic properties despite repeated washings. In fact, improved physical properties of the fabric as a result of this treatment permit it still to exert antimicrobial effects after a number of washings sufficient to weaken and disintegrate untreated control fabrics. At the same time, the treatment of this invention does not detrimentally affect such physical properties of cloth, fibers and sheet material as smoothness, flexibility, softness in "hand," washability and wettability.

For treating articles under near-neutral or acidic conditions, boric acid, borax, alkali-metal acetates (e.g. the acetates of sodium, potassium or lithium) and other common buffering agents as well as mixtures thereof are advantageously added. Any of the commercially available textile surfactants of the ionic, especially quaternary, or non-ionic types will serve as the wetting agent or detergent, including, for example, the various sulfonated long-chain alcohols and esters as well as phenolates, sorbates, quaternary ammonium salts or naphthenates. The use of quaternary ammonium salts has been found to be especially advantageous in the treatment of nylon. The following compounds are illustrative of the detergents which may be employed:

## TABLE A

## Non-Ionic Detergents

- 60 Sorbitan sesquioleate (Arlacel C)  
Polyethanolamine condensate of a fatty acid (Cerfak N-100)  
Alkoxypolyglycol fatty-acid ester (Dergon PX)  
Sulfated glyceryl trioleate (Drutone SE)  
65 Polyoxyethylene alkyl phenol (Energetic W-100)  
Fatty-acid condensate of N-methyl glucamine and coconut fatty acids (Glucaterge 12)  
Isocetyl phenoxy polyoxyethylene ethanol (Igepal CA 630)  
70 Nonyl phenoxy polyoxyethylene ethanol (Igepal CO 633)  
Polyoxyethylene sorbitol stearate (Morosol SL)  
Polyoxyethylene stearate (Myrij 45)

## Quaternary Detergents

Alkyl (fatty acid) benzyl dimethyl ammonium chloride (benzalkonium chloride)

Tallow trimethyl ammonium chloride (Arquad-T)

Soya trimethyl ammonium chloride (Arquad-S)

Dodecyl trimethyl ammonium chloride (Arquad 12)

Representative water-soluble zinc salts useful in the composition of the invention include zinc chloride, zinc bromide, zinc nitrate, zinc sulfate and zinc acetate. As sequestrants or chelating agents the alkali-metal (e.g. sodium, potassium, lithium) salts of the following acids may be employed herein: ethylene diamine tetracetic acid, methylimino diacetic acid, phenylimino diacetic acid, ammonia triacetic acid, 1,2-diamino-cyclohexanetetraacetic acid and uramildiacetic acid. Of these, sodium salt of ethylene diamine tetracetic acid has been found particularly advantageous in view of its ready availability and low cost.

In general, any amine source soluble in the treatment medium may be used, provided that its dissociation constant ( $K_b$ ) is greater than  $1 \times 10^{-14}$ .

Such amines include the following:

TABLE B

|                   |                    |
|-------------------|--------------------|
| Urea              | Triethanolamine    |
| Isopropylamine    | Aniline            |
| n-Propylamine     | Toluidine          |
| t-Butylamine      | p-Phenylenediamine |
| Monooethanolamine | Morpholine         |
| Diethanolamine    | Melamine           |

An initial mixture of zinc salt, sequestrant, buffering agent and detergent (with or without aminating agent), which can itself serve as an article of commerce, may be prepared either in dry granulated form or as a liquid concentrate. To manufacture the former, the dry ingredients are mixed together and granulated in known manner. To form the treatment bath, a requisite amount of the granulated product is dissolved whereupon the liquid concentrate may be diluted to a desired extent. The bath is brought to an elevated temperature and the material to be treated is immersed in it. The proportion of concentrate in the bath depends on the amount of zinc-amine complex it is desired to incorporate into the final product. In general, a good practice is to utilize from 0.5% to 35% by weight of the concentrate in the treating bath to obtain optimum results, 1% to about 10% being preferred.

Further control of the deposition of the zinc-amine polymer in the fiber may be effectuated by the degree of wetting and the curing temperature used to fix the complex in the fibers. A measure of the degree of wetting and penetration of the reactants is the "pick-up" of bath liquid by the fibers. This pick-up is defined as the percentile of the difference between wet and dry weights to the dry weight of the fibers. The greater the degree of pick-up the lower the necessary initial concentration of the complexing agent. Generally, higher fixing temperatures result in a firmer bonding of the zinc complex to the polymeric molecule of the treated material.

It has further been determined that the process and the baths used therein are compatible with the various "wash and wear" treatments presently applied to textiles. These known treatments consist in the impregnation of the textile with polymeric resinous materials of either the thermoplastic or the thermosetting type. The thermoplastic treatment resins are usually applied in the form of emulsions, while the thermosetting-type materials are applied in the form of aqueous solutions of the resin prepolymers which are subsequently set in the fabric by the application of heat. The treatment of this invention can be carried out before or during the application of the "wash and wear" treatment without loss in effectiveness of either treatment.

The single-step process of treatment according to the

invention is most efficiently practiced in aqueous baths with the various components present in the following concentrations:

|                                              | Percent   |
|----------------------------------------------|-----------|
| 5 Chelating agent or sequestrant             | 0.1 to 10 |
| Water-soluble organic or inorganic zinc salt | 0.5 to 50 |
| Aminating agent                              | 0.5 to 30 |
| Detergent or wetting agent                   | 0 to 15   |
| Buffering agent                              | 0 to 25   |

10 If the invention is to be practiced as a two-step process, a granulated mixture comprising the soluble zinc salt, a detergent and a sequestrant is advantageously prepared for dissolution in an aqueous medium constituting a first treating bath; next, a second aqueous bath comprising 15 from 0.5% to 30% of the above-mentioned aminating or fixing agent is produced. In general, the reactive proportions of the ingredients of the granulated mixture introduced into the first bath may vary, in the dry state, within the following ranges:

|                 | Percent |
|-----------------|---------|
| 20 Zinc salt    | 20-90   |
| Sequestrant     | 2-30    |
| Detergent       | 0-30    |
| Buffering agent | 0-40    |

25 For optimum antimicrobial action, however, it is found that the preferred ranges are approximately 50%-70% for the zinc salt, 2.5%-10% for the sequestrant, 3-10% for the detergent and 15%-30% for the buffering agent.

30 In many instances, it will be found desirable to invert the order of the two baths listed above, by first pretreating the fabric or other organic film or fiber material with the aminating agent and subsequently immersing said material, while still wet, in the active zinc-containing bath 35 composed as indicated above.

40 More specific modes of operation will be described in the following examples. It is to be noted that the examples only represent preferred modes with regard to the specific material set forth. Departures from the specific formulations may be necessitated by changes in the material to be treated, time or temperature. Unless otherwise specified, the parts given are by weight.

## EXAMPLE 1

[Additive A]

|                                                                                                                                        | Parts |
|----------------------------------------------------------------------------------------------------------------------------------------|-------|
| 45 Tetra-sodium salt of ethylene diamine tetra-acetic acid (E.D.T.A.)                                                                  | 1     |
| Zinc chloride                                                                                                                          | 22    |
| Sodium acetate                                                                                                                         | 5     |
| 50 Boric acid                                                                                                                          | 1     |
| Ethylene cycloimido, 1 alkyl (fatty acid), 2 hydroxy ethylene sodium alcoholate, methylene sodium carboxylate (Miranol CM concentrate) | 2     |
| Urea                                                                                                                                   | 31    |

55 Thirty grams of the above mixture is dissolved in a liter of water to form the treatment bath. The bath is heated to 70° C. and knitted cotton socks are immersed in the bath for 10 minutes and then extracted, rinsed in water and dried. Tests indicate that contact with the treated socks inhibits growth of test bacteria. Moreover this inhibiting quality continues in the socks even after they have been subjected to as many as fifty automatic-washing-machine cycles. Untreated control socks do not display any inhibiting properties, yet it is noted that 20% of the controls showed tears due to the wear resulting from this washing procedure alone. Treated socks do not tear.

60 Similar results are obtained when zinc acetate is employed in lieu of zinc chloride to formulate the additive according to Example 1.

## EXAMPLE 2

65 Fifteen gms. of additive A (Example 1) is added to 600 cc. of a prepared resin bath, as conventionally used 70 in the "wash and wear" treatment of cotton fabrics, and

the mixture is agitated until the additive is completely dissolved therein.

The fabric to be treated (shirting) is immersed in the resulting solution at room temperature, until it is completely wetted (30-60 seconds), and is then removed from the bath. The fabric is drained or pressed until the pick-up of the bath by the fabric is 70%-120%. The fabric is then dried at, for example, 120° C. for one minute and washed in a softening bath containing a detergent such as, for instance, polyglycol monolaurate or monostearate. Tests show inhibition of bacterial growth by contact with the treated fabric. This property of the treated material is observed after the treated fabric is subjected to 50 washing cycles in standard soaps. Untreated controls possess no inhibitory properties either before or after the washing cycles. Similarly, shirtings treated with the "wash and wear" resins without the additive are found to have no anti-bacterial properties.

## EXAMPLE 3

[Additive B]

|                                     | Parts |
|-------------------------------------|-------|
| Tetra-sodium salt of E.D.T.A. ----- | 1     |
| Zinc chloride -----                 | 22    |
| Sodium acetate -----                | 5     |
| Boric acid -----                    | 1     |
| Urea -----                          | 31    |
| Sorbitan sesquioleate -----         | 2     |

Fifteen grams of additive B are dissolved in a liter of water, at 70° C. Woolen socks are immersed in the solution until they absorb 90 to 120% of their weight of the solution. The socks are then heated to 50° C. and maintained at or above that temperature for at least 15 minutes or until the socks are dry. The residue of the bath is then washed or rinsed from the socks. The so treated socks maintain their anti-microbial properties through 30 washing cycles. Controls exhibit no microbe-inhibiting characteristics either before or after the washing. When the di-potassium salt of methylimino diacetic acid is substituted for the tetra-sodium salt of ethylene diamine tetraacetic acid, similar results are observed.

## EXAMPLE 4

A bath according to Example 3 is used for the processing of cotton-polyester (Dacron) 65-35 shirting. The shirting is immersed for 2 minutes in the bath at 40° C. until the dry-weight "pick-up" of the bath by the shirting is 70%. The fabric is then dried at 80° C. The finished fabric (after rinsing and drying) inhibits growth of bacteria in direct contact with it before and after 40 wash cycles.

## EXAMPLE 5

Rayon tricot fabric is treated in the manner set forth in Example 3 except that the fixing and drying is carried out between 60° and 80°. The fabric exhibits bacteria-inhibiting properties before and after 30 wash cycles.

The following examples illustrate the two-step treatment according to the present invention:

## EXAMPLE 6

|                                                             | Parts |
|-------------------------------------------------------------|-------|
| Tetra-sodium salt of ethylenediamine tetraacetic acid ----- | 1     |
| Miranol CM concentrate (cf. Example 1) -----                | 2     |
| Sodium acetate -----                                        | 5     |
| Boric acid -----                                            | 1     |
| Zinc chloride -----                                         | 22    |

The above mixture granulates easily and is stable in granulated form. Five parts of the above dissolved in 200 parts of water yields a solution having a pH of about 6. Diverse cellulosic materials such as sheets of regenerated cellulose and cellulose sponges when immersed in a bath of this solution at its boiling point for a period of 10 minutes or longer exhibit on analysis a zinc content up to about 3% by weight, depending on the time

in the bath and the pick-up rate. Such materials, without further fixing, retain their antimicrobial properties up to approximately 10 washings.

## EXAMPLE 7

5 The products of Example 6, having a zinc content of 3%, are fixed by immersion in a 2½% solution of urea at 80° C. for 5 minutes. A specific product so treated, hospital sheeting, maintains its antimicrobial properties after 50 washings against common skin bacteria as shown by inhibition zones in the standard agar Petri-dish test.

## EXAMPLE 8

15 The products of Example 6, having a 2% zinc content, are fixed by immersion, for 7 minutes at 65° C. in a bath containing 3% monoethanolamine. Handkerchiefs treated in this manner maintained their antimicrobial properties over periods of prolonged use and many washings.

20 In lieu of monoethanolamine, morpholine can also be used as the aminating agent.

## EXAMPLE 9

|                                         | Parts |
|-----------------------------------------|-------|
| Tetra-sodium salt of E.D.T.A. -----     | 1     |
| Polyoxyethylene sorbitol stearate ----- | 1     |
| Sodium acetate -----                    | 5     |
| Borax (tetrasodium borate) -----        | 2     |
| Zinc chloride -----                     | 10    |

30 The above mixture granulates easily by the interchange of the water of crystallization between the borax and the zinc chloride. One part of the above mixture dissolved in 9 parts of water yields a protein-treating bath, having a pH of approximately 8. A proteinaceous material, such as wool, silk, leather, or catgut sutures, when immersed in 35 the above treatment bath for preferably not less than 10 minutes absorbs within the protein molecule up to 4% of zinc. The zinc may be fixed permanently within the molecule by any of the fixing baths mentioned in connection with the cellulosic materials (Examples 7 and 8) with 40 similar antimicrobial results. It should be noted that proteins are preferably treated at lower temperatures but for longer treatment times. Woolen fabrics after 13 minutes in the above treating solution at 65° C. have a zinc content in excess of 1% fixed within the fabric. Moreover it has been noted that dyed treated fabrics possess greater resistance to actinic rays than the same dyed fabrics without said treatment.

## EXAMPLE 10

50 Cellulosic materials as mentioned in Example 6 or proteinaceous materials as set forth in Example 9 are first immersed for 5 minutes in a urea solution as mentioned in Example 7. This treatment is immediately followed by immersion in a bath as described in Example 6. The 55 wash resistance of the treated material is at least equal to that of the product of Example 7.

The process of Example 10 may be modified by substitution of the ingredients of Example 8 and/or 9 for those listed in Examples 6 and 7.

60 The presence of chelating agent appears to have the dual effect of facilitating the introduction of the zinc into the molecules of the organic base material and detoxicating the resultant product by rendering harmless any excess zinc salts which might otherwise be left in contact therewith.

65 The use of a two-step process for the treatment according to the present invention has the advantage of appreciably shortening the time during which the material to be treated will remain immersed. Thus, immersion times of 70 as little as a few seconds per bath have been found suitable in many instances, in contradistinction to an immersion time upwards of approximately five minutes for the sole bath of the one-step process. It may also be mentioned that the time interval elapsing between the successive immersions of the two-step process is not critical and may

range from about a second to a week or longer, any intervening drying of the treated material being of no apparent consequence regardless of the order in which the two steps are applied. Thus, the two-step treatment lends itself particularly for use in commercial processing plants, where long webs of fabric or the like could be treated in a continuous operation or where piece goods could be immersed in baths for short periods, whereas the one-step treatment will be preferable for small laundries and home washing machines.

We have found that, for reasons not fully understood, bath compositions including a combination of two detergents, one from the non-ionic group and the other from the quaternary group of Table A, are particularly effective if the treatment is to be applied to films or fibers not readily wettable in aqueous solution, such as polyamides (nylon). The foregoing examples may, accordingly, be modified for such purposes by replacing a fraction (preferably one-half) of the detergent of one type by a like amount of detergent of the other type.

Whereas the treatment previously described is most expeditiously carried out at immersion temperatures ranging between 60° C. and 100° C., followed (if desired) by a forced drying at even higher temperatures if the treated material can be safely subjected thereto, we have found that, in accordance with a further feature of the invention, the process can be performed at considerably lower temperatures (upwards of about 45° C.) if a small percentage of a natural or synthetic gum is admixed with the active bath. This class of additives includes polyvinyl alcohol; water-soluble polyuronic acids and derivatives thereof, such as alginic or pectinic acid and their sodium or potassium salts; and water-soluble cellulose ethers such as methyl cellulose, carboxymethyl cellulose or hydroxyethyl cellulose.

The quantity of temperature-lowering additive (gum) may range upwards of about 1%, by weight, of the solids; the upper limit is given by the proportion which will tend to make the bath too viscous for effective immersion of the article to be treated, such proportion being generally in the vicinity of 5% of the liquid or up to about 50% of the solids, depending upon the total ratio of solids to liquid which may range between 0.1% and 25% but is preferably held within the limits of 1% and 10%, by weight.

#### EXAMPLE 11

The composition of Example 1 (additive A) is supplemented by 10 parts of polyvinyl-alcohol powder. Cotton goods (e.g. socks) are immersed for ten minutes as specified above, but at a temperature of 50° C. The treatment is otherwise the same as that previously described, with closely similar results.

In like manner the compositions of the treatment bath of Example 3 or of the active baths listed in Examples 6 and 9 may be fortified with polyvinyl alcohol or with any of the other gums mentioned above.

The addition of such gums is believed to counteract any tendency of the active ingredients to settle out of the bath at lower temperatures, and to help attach the zinc complex to the treated material under conditions which might otherwise not lead to an effective fixing thereof by the aminating agent. We have, moreover, discovered that

the number of permissible washings is increased by this addition, on the average, by 20 to 30%.

The preferred pH for the active bath of the two-step process or the combined bath of the one-step process according to the invention ranges substantially between 5 and 7. The extended operative range of the pH is from 3 to 9. Alkaline solutions with a pH greater than 10 should be avoided.

We claim:

10. An antimicrobial composition comprising a zinc salt, an aminating agent and a chelating agent.
2. A composition according to claim 1 including a buffering agent.
3. A composition according to claim 1 including a wetting agent.
15. An antimicrobial composition comprising a zinc salt selected from the group consisting of zinc chloride, zinc bromide, zinc nitrate, zinc sulfate and zinc acetate; urea; and an alkali metal salt of ethylenediaminetetraacetic acid.
20. 5. As an article of manufacture, textile fiber impregnated with a composition comprising a zinc salt, an aminating agent and a chelating agent.
6. An article of manufacture according to claim 5
25. 25 wherein said textile fiber is selected from the group consisting of cellulosic, proteinaceous, nylon and polyester fibers.
7. A composition of matter comprising from .5% to 50% by weight of a water-soluble zinc salt, 1% to 10% by weight of a chelating agent and from .5% to 30% by weight of an aminating agent.
30. 8. A composition of matter according to claim 7 containing up to 15% by weight of a surfactant.
9. An antimicrobial composition comprising zinc chloride, tetraalkali metal salt of ethylenediaminetetraacetic acid and urea.
35. 10. A process for imparting antimicrobial properties to textile fibers comprising applying in solution to said fibers a zinc salt, an aminating agent and a chelating agent, whereby antimicrobial properties are imparted to said textile fibers.
11. A process for imparting antimicrobial properties to textile fibers comprising applying to said fibers a solution of a zinc salt and a chelating agent and subsequently subjecting the fibers so treated to the action of an aminating agent whereby antimicrobial properties are imparted to said textile fibers.

#### References Cited in the file of this patent

#### UNITED STATES PATENTS

- |           |                |       |                |
|-----------|----------------|-------|----------------|
| 2,304,478 | Rosenzweig     | ----- | Dec. 8, 1942   |
| 2,396,514 | Kreidl et al.  | ----- | Mar. 12, 1946  |
| 2,459,896 | Schwarz        | ----- | Jan. 25, 1949  |
| 2,459,897 | Schwarz        | ----- | Jan. 25, 1949  |
| 2,525,049 | Signaigo       | ----- | Oct. 10, 1950  |
| 2,527,141 | Mantell et al. | ----- | Oct. 24, 1950  |
| 2,572,923 | Gaver et al.   | ----- | Oct. 30, 1951  |
| 2,609,368 | Gaver          | ----- | Sept. 2, 1952  |
| 2,648,593 | Stanton et al. | ----- | Aug. 11, 1953  |
| 2,671,779 | Gaver et al.   | ----- | Mar. 9, 1954   |
| 2,868,724 | Zech           | ----- | Jan. 13, 1959  |
| 2,904,468 | Davis et al.   | ----- | Sept. 15, 1959 |